

# UNITED STATES PATENT OFFICE.

CHARLES HOWARD SMITH, OF SHORT HILLS, NEW JERSEY, ASSIGNOR TO INTERNATIONAL COAL PRODUCTS CORPORATION, OF RICHMOND, VIRGINIA, A CORPORATION OF VIRGINIA.

## FUEL-BRIQUET.

1,284,939.

Specification of Letters Patent. Patented Nov. 12, 1918.

No Drawing. Original application filed November 15, 1916, Serial No. 131,434, (now Patent No. 1,276,429, dated August 20, 1918.) Divided and this application filed July 18, 1918. Serial No. 245,455.

*To all whom it may concern:*

Be it known that I, CHARLES HOWARD SMITH, a citizen of the United States and a resident of Short Hills, in the county of 5 Essex and State of New Jersey, have invented certain new and useful Improvements in Fuel-Briquets, of which the following is a specification.

The invention relates to briquets and in its 10 broader aspect it is directed to briquets composed principally, if not wholly, of partially carbonized coal and in which the hydrocarbon volatile content of the briquet is approximately from eleven per cent. 15 (11%) to seventeen per cent. (17%) of the weight of the briquet.

According to a more specific aspect of the invention it is directed to briquets made principally from partially carbonized coal 20 but, also including hydrocarbon binding material, such as pitch. In the making of the briquets just referred to uniformly but partially carbonized coal having a hydrocarbon volatile content of generally less 25 than ten per cent. (10%) to eleven per cent. (11%) is employed. Pitch or other suitable hydrocarbon binding material is mixed with this partially carbonized coal until the hydrocarbon volatile matter in the mixture of the 30 partially carbonized coal and hydrocarbon binder approximates the desired amount, as from eleven per cent. (11%) to seventeen per cent. (17%). Said mixture is formed into a mash preferably as by the aid of 35 steam which may be employed during a fluxing operation and from this mash the desired pressed briquets are made by molding.

The invention which is the basis of the 40 present application is clearly described in my United States Letters Patent No. 1,276,429 dated August 20, 1918, entitled "Briquets and method of making the same." The present application is a division of said 45 patent.

The briquets which are the basis of the present invention can be readily made from a high volatile fuel, for example, a raw coal having as high as thirty-six per cent. (36%) 50 volatile matter and fifty-five per cent. (55%) of fixed carbon. They can be employed as raw briquets but they are particularly adaptable for use in the making of carbonized briquets wherein the volatile content

of the final briquet is as low as two and one-half per cent. (2½%) or less. By proper heat treatment these final briquets can be made so as to each have a firm, coherent structure and with the percentages of volatile matter above mentioned. By the proper heat treatment the final briquets will have the same shape as the raw briquets, although it will be noted that a substantial shrinkage takes place during said heating which is a carbonizing operation. One way in which the 60 briquets can be made having approximately eleven per cent. (11%) to seventeen per cent. (17%) volatile matter is as follows:

Raw coal having about thirty-six per cent. (36%) volatile matter and fifty-five 65 per cent. (55%) fixed carbon may be heated in a retort, preferably progressively and uniformly throughout, until a maximum temperature varying approximately from 825 degrees F. to 1200 degrees F. is reached 70 and during which heating tar vapors in the coal are largely removed. During said heating the coal is preferably mixed and agitated in such a manner that the resulting product from the retort is a dry, soft, uniformly distilled or partially carbonized coal residue, or semi-coke as some might call it. This residue at the end of the heating operation 75 may, for example, contain only five per cent. (5%) hydrocarbon volatile matter therein. 80 It is not necessary, however, to carry the heating to a point where the volatile matter will be lowered to the percentage just mentioned, as the point where the heating is stopped is dependent more or less upon 85 the coal being treated and the product desired for the making of the particular briquet required.

This coal residue is rendered in finely divided or pulverized form, as by crushing, 95 and to it there is added pitch, for example crushed pitch in finely divided form, until in the resulting mixture there is contained hydrocarbon volatile matter which approximates from eleven per cent. (11%) to 100 seventeen per cent. (17%), the amount of pitch added being dependent upon the percentage of hydrocarbon volatile matter in the partially distilled coal residue that enters into the briquet and also upon the percentage of hydrocarbon volatile matter that is desired in the resulting or raw briquet.

The mixture may be fluxed by the aid of

steam and it will here be noted that the pitch can be added during the fluxing operation or previous thereto. Other hydrocarbon bearing materials than pitch could be employed to supply this volatile hydrocarbon binder. The result of the fluxing operation is a mash. The word "mash" used herein is employed to designate a mass of crushed or finely divided partially distilled coal having intermixed therewith water or hydrocarbon volatile matter in liquid or plastic form whereby there results a soft mixture of plastic material that can be readily molded into briquets. The mash is then formed by pressure into briquets having the desired size and shape and thereafter these briquets can be employed either directly, as for the purpose of supporting combustion, or they can be carbonized to make the firm, coherent, low volatile carbonized briquets previously referred to.

While the partially carbonized coal employed in the making of raw briquets is described above as being made from high volatile coal, still it will be manifest that the invention is not limited to the employment of partially carbonized coal resulting from the heating of a high volatile coal, as coals having less hydrocarbon volatile could be employed to provide the partially carbonized coal in case they contained enough hydrocarbon volatile to permit the preliminary partial carbonization or distillation necessary to produce the desired coal residue from which to make the raw briquets.

According to a broader aspect of the invention the carbonizing of the raw coal may be only enough to leave in the coal approximately from eleven per cent. (11%) to seventeen per cent. (17%) hydrocarbon volatile matter whereby the necessity for adding hydrocarbon volatile matter, such as pitch, could be avoided. In such a case, however, this partially carbonized coal might be rendered in finely divided form and made into raw briquets having the desired percentage of hydrocarbon volatile matter therein whereby the desired results can be realized, although it will be understood that, according to the preferred or

more specific embodiment of the invention, employment is made of the pitch which has many qualities that are advantageous in briquets of the kind in question.

It will be manifest that the invention can be readily realized in various forms and ways without departing from the spirit and scope thereof.

What I claim is:

1. A briquet formed of a partially carbonized coal and binder, as pitch, and having a volatile content of approximately from eleven per cent. (11%) to seventeen per cent. (17%).

2. A briquet formed largely of partially carbonized coal and in which the hydrocarbon content of the briquet approximates from eleven per cent. (11%) to seventeen per cent. (17%).

3. A briquet comprising partially carbonized coal which provides fixed carbon and hydrocarbon volatile matter and mixed therewith hydrocarbon binding material which provides hydrocarbon volatile matter so that the hydrocarbon volatile matter in the briquet approximates from eleven per cent. (11%) to seventeen per cent. (17%) of the weight of the briquet.

4. A briquet which comprises partially distilled coal and which briquet has from eleven per cent. (11%) to seventeen per cent. (17%) hydrocarbon volatile matter therein.

5. A briquet comprising finely divided uniformly but partially distilled coal residue with which there is mixed pitch until the hydrocarbon matter in the mixture approximates from eleven per cent. (11%) to seventeen per cent. (17%).

6. A briquet having dry, soft, finely divided, partially carbonized coal residue and in which briquet the percentage of hydrocarbon volatile matter approximates from eleven per cent. (11%) to seventeen per cent. (17%).

This specification signed and witnessed this 17th day of July, 1918.

CHARLES HOWARD SMITH.

Signed in the presence of—

G. MCGRANN,  
W. C. MARGESON.